

## UNITED STATES PATENT OFFICE

2,410,770

## BENEFICIATION OF FLUORITE

Robert B. Booth, Springdale, and Joseph E. Carpenter, Greenwich, Conn., assignors to American Cyanamid Company, New York, N. Y., a corporation of Maine

No Drawing. Application August 23, 1943,  
Serial No. 499,693

8 Claims. (Cl. 209—166)

1

This invention relates to the beneficiation of non-siliceous minerals. More particularly, the invention relates to an improved method of concentrating fluorite by froth flotation from ores containing fluorite, barite, calcite and other like non-siliceous minerals, as well as siliceous minerals.

Concentration of fluorite from fluorite-containing ores in which the remaining constituents are principally non-metallic, non-siliceous minerals constitutes an industrially important operation. Extensive installations for carrying out this operation by froth flotation are in regular use. Theoretically, the beneficiation of fluorite ores by froth flotation should be quite simple since the pure mineral itself is readily floated by the use of so-called "anionic" flotation reagents such as for example the fatty acids, talloel and the like as well as the various soaps thereof. Unfortunately however, the gangue constituents of many fluorite-containing ores are also readily collected by the same reagents. As a consequence, considerable work has been done to develop satisfactory methods of carrying out the operation. A number of such processes have been proposed. Some have been practically useful, others have not.

Of these proposed methods, those which have produced acceptable results have usually involved heating the ore-pulp which is to be subjected to froth flotation. Heating the pulp apparently serves the double purpose of aiding in procuring proper dispersion of the flotation reagents and in improving their selectivity. In common practice, the pulp is heated to a temperature in the range of about 80-100° F. Without heating, an acceptable concentration is not only very difficult to obtain, but at the same time, the reagent consumption is usually excessive.

Limiting a process to elevated temperatures in this way is a serious drawback, both from the point of view of added expense and from the point of view of ease in operation. The objectionable features of the practice are particularly aggravated during cold weather, when the water supply is necessarily at a low temperature. Despite the obvious inconveniences of heating, it has continued to be regarded as necessary for successful operation.

There remains therefore an unsatisfied demand for a process of beneficiating fluorite which is not subjected to these difficulties, i. e., one which is not particularly sensitive as to the amounts of reagents used and does not require heating the pulp in order to obtain successful beneficiation.

It is, therefore, the principal object of the present invention to provide one such process. It is also an object of the present invention to provide a novel reagent combination which not

2

only will permit carrying out the operation without heating, but which will produce an equally good or better beneficiation at low temperatures than that previously obtainable with comparable amounts of the usual reagents, even when the latter are used in a heated pulp.

In general, the objects of the present invention are accomplished by the use of a flotation reagent comprising sulfonated petroleum hydrocarbons of the green acid type obtained in the refining of petroleum lubricating oils or salts or soaps of such acids. In addition, a suitable depressant for the calcite and the like minerals is ordinarily used. In order to obtain optimum results, certain ores are preferably conditioned with the reagents at high solids prior to the actual froth flotation.

Sulfonated petroleum hydrocarbons, such as those which constitute the principal reagent in carrying out the novel process of the present invention, are commercially available in a number of different forms. However, as shown, for example, in U. S. Patent 2,331,049, their principal source is as by-products from the refining of petroleum lubricating oil fractions in the course of treatment with fuming sulfuric acids or sulfuric acids. When so produced, these by-products are generally found to be salts of the sulfonated hydrocarbons. Most commonly, the metallic radical of the salt is sodium. However, salts of other metals such as the alkaline earth metals, aluminum and the like are encountered. In some cases, no attempt has been made to neutralize the acid product. Even after neutralization, free sulfonates and/or sulfates are often found.

So far as the present invention is concerned, it makes little difference whether the sulfonated petroleum hydrocarbon is used per se or as a salt; whether or not the sulfur is present in a sulfate or a sulfonate group, there usually being some of both present; or whether the compounds are used as salts of sodium, potassium, calcium, barium, aluminum and the like. Nor need the materials be purified, since mixtures of compounds produce wholly satisfactory results. As used in the present case, the term "sulfonated petroleum hydrocarbons" is therefore intended to include such mixtures as are found in the commercial products.

Petroleum sulfonates, or derivatives thereof, which are suitable for use according to the process of the present invention are commercially available under a variety of designations. Among these found to be useful are "Petronate" and "O-Emulsifier," obtainable from L. Sonneborn Sons; "Eldrol" and "Petrosul," obtainable from Pennsylvania Oil Products Refining Co.; Sherwood "Reagent 407," obtainable from Sherwood Refining Co.; "Ultranan #2," obtainable from Atlantic Refining Co.; and "SP-1," "SP-302," and

"SP-312," obtainable from Stanco Distributors, Inc.

However, the commercially-available, sulfonated petroleum hydrocarbons may be divided on a functional basis into two distinct groups. One of these is the group variously known as "mahogany" acids, "mahogany" soaps and the like. This group is characterized in that its constituents are generally oil-soluble but water-dispersible. Usually, but not necessarily, these compounds have a deep mahogany color when in solution which gives rise to the generic designation as "mahogany" compounds.

The other group is generally, but not necessarily, characterized by a green coloration in solution. Hence, compounds of this group are usually referred to as "green sulfonic" acids or "green" soaps. More important than the color distinction however, is the fact that the so-called "green" compounds are characterized by being water-soluble. Despite their other similarities the two groups of compounds are by no means necessarily equivalents each to the other. Particularly is this true as in the present invention, when they are applied to ore dressing problems.

The instant application is primarily concerned with the use of the water-soluble petroleum sulfonates, i. e., the green sulfonic acids and salts or soaps thereof, which require considerably different treatment than those of the "mahogany" or oil-soluble type.

In general, the process of the present invention comprises the steps of reducing the ore to a size suitable for feed to a froth flotation operation; desliming the ore, if necessary; making a pulp of the ore with water; adding the reagents thereto; subjecting the pulped ore to froth flotation and finally collecting the froth concentrate in the usual manner.

Where it is desirable to use a desliming operation, it has been found well in some cases to carry out this operation in the presence of soda ash or some equivalent alkaline material to assist in freeing the slimes. If a depressant for the gangue is to be used in the subsequent operations, it is also well to add a small amount of the depressant during desliming. Where a depressant for the gangue minerals is to be used in carrying out the process of the present invention, quebracho was found to give excellent results. Other depressants such as dextrin, particularly yellow corn dextrin, and the alkali phosphates and polyphosphates may be used with highly satisfactory results. In some cases no depressant is necessary.

It was also found desirable in certain cases to condition the ore-pulp with the flotation reagents prior to the actual flotation step. Pulp densities of about 60-65% solids were found to give excellent results and to be ordinarily preferable. However, if so desired, lower pulp densities even down to densities such as those commonly used in flotation operations *per se* may be used. The invention is not necessarily limited to any particular mode of admixture, and the reagents may be added directly to the flotation cell if so desired and still obtain acceptable results.

The green type of petroleum sulfonates and/or their derivatives which are used in the present process are characterized, as noted above, by their solubility in water. While this solubility is not always complete, it is sufficiently high so that when used alone the reagent may not always produce the optimum concentration of fluorite. These green compounds appear to lack certain water-repellant properties which are helpful in

making successful concentration. In the process of the present invention, this difficulty is readily overcome by the addition of an amount of a more hydrophobic material. This may be done by adding an oil in suitable quantity or by mixing some of the oil-soluble petroleum sulfonates with the water-soluble type. Any of the commercially available oils of animal, vegetable or mineral origin may be used for this purpose. Unsulfonated petroleum derivatives such as crude oil, kerosene or fuel oil are very suitable. Saponifiable oils, such as cocoanut oil, cotton seed oil and other glyceride oils may be used. Anionic materials such as the fatty acids and the like also may be used, provided the gangue constituents are such as not to be floated by these materials. Tallow, in view of its low cost, is especially useful.

Amounts of these materials used will obviously vary with the particular circumstances. The most pronounced variations in demand are caused by the nature of the ore and the particular water-soluble petroleum sulfonates being used. No general rule can therefore be empirically established for all cases. In general, however, the amounts required have been found to fall within the range of about 0.1-2.5 lbs./ton of ore treated. Ordinarily however, the amounts used will be between about 0.5 and 1.5 lbs./ton. Variations in the temperature at which the flotation is carried out have also been found to have an effect on the amount of these hydrophobic materials required.

Similarly, the nature of the ore, the temperature, the pulp density, the water used, the source of the water-soluble petroleum sulfonates and the amount of slimes present, all have been found to have a direct bearing on the amount of water-soluble petroleum hydrocarbons required to bring about an effective concentration of the mineral value. Therefore, as in the case of the hydrophobic materials, no fixed rule applicable to all instances can be laid down as to the amount of collecting agent required. In general, however, it has been found that amounts of water-soluble petroleum hydrocarbons ranging from about 0.1 to 5.0 lbs./ton will take care of all but the most extraordinary cases. With the ores most commonly encountered, this range can be substantially halved, since most of the ores may be readily beneficiated using an amount of reagent in the range from about 0.2 to 2.5 lbs./ton.

As has been shown, the water-soluble petroleum sulfonates have generally proved to be satisfactory when used as the principal promoter for the fluorite minerals. However, certain external circumstances may require that the actual froth flotation operation be carried out in the presence of other substances such as oleic acid, tallow and the like which are themselves well known anionic-type reagents. This condition may be brought about by the nature of the flow scheme employed, the presence of these additional agents being due to other operations which are being carried out in the same plant. For example, these reagents are frequently carried along in reusing process water. It has been found that the water-soluble petroleum sulfonates are perfectly effective in the presence of these extraneous reagents. In fact, as has been noted above under some circumstances, these agents may be added deliberately in order to replace all or part of the oil normally used to overcome any difficulty which may arise due to the solubility of the sulfonated petroleum hydrocarbons. Similarly, the presence of small

amounts of the water-soluble petroleum sulfonates has been frequently found to increase the effectiveness of these additional reagents in their intended applications.

There is, however, a marked advantage of the present invention in that equally good or better results can be obtained at low temperatures than are normally obtained in prior practice at high temperatures. This feature of the invention will be more fully illustrated in connection with the following examples which are meant to be illustrative only and not by way of limitation. All parts are by weight unless otherwise noted. "Tons" as used in the following examples refer to short tons.

EXAMPLE 1

An Illinois fluorite ore, containing chiefly fluorite (about 72%  $\text{CaF}_2$ ) and limestone (about 18.5%  $\text{CaCO}_3$ ), was ground to minus 65 mesh and deslimed using 2 lbs./ton of soda ash and 0.1 lb./ton of quebracho. The deslimed pulp was then made up to 22% solids and conditioned for 1 minute with about 0.1 lb./ton of quebracho and varying amounts of green acids. In different tests the pulp was treated at different temperatures. The conditioned pulp was subjected to froth flotation in a Fagergren Flotation Machine. The concentrate was cleaned once using 0.25 lb./ton of quebracho. It was found that acceptable results could be obtained using green acids in amounts varying from 0.5-2.0 lbs./ton over a temperature range of from 32-100° F. At the lower temperatures it was found that slightly more reagent was required, that the recovery was slightly less but that the concentrate in general was of higher grade and contained less objectionable non-metallic gangue. Illustrative results are shown in Table I.

Table I

|                                                    |       |       |
|----------------------------------------------------|-------|-------|
| Temperature, °F.                                   | 86    | 32    |
| Lb./ton—green acids                                | 1.00  | 1.50  |
| Lb./ton—fuel oil                                   | 1.00  | 1.50  |
| Cleaner conc.—per cent $\text{CaF}_2$ assay        | 93.58 | 94.76 |
| Cleaner conc.—per cent $\text{CaCO}_3$ assay       | 4.84  | 3.96  |
| Cleaner conc.—per cent $\text{CaF}_2$ distribution | 71.33 | 68.65 |
| Cleaner tailing—per cent $\text{CaF}_2$ assay      | 67.58 | 73.24 |
| Rough tailing—per cent $\text{CaF}_2$ assay        | 14.60 | 42.00 |

As was noted above the presence of mahogany soap in addition to the green type of compounds permitted excellent beneficiation operations to be carried out using none of the oil or fatty acid which was found to be important when green acids alone were used. An illustration of this type of operation is shown in the following example.

EXAMPLE 2

An additional sample of the same ore treated in Example 1 was ground and deslimed in the same manner. Portions of the deslimed ore were then subjected to the conditioning operation at about 65% solids with varying amounts of Hydroll R (a commercial mixture of water-soluble and oil-soluble petroleum sulfonates obtainable from Emery Industries Inc.) which was diluted with secondary butyl alcohol in the proportion of

10 to 1. This conditioned pulp was subjected to froth flotation in the Fagergren Flotation Machine at room temperature as in Example 1. Illustrative results are shown in Table II.

Table II

|                                                    |       |
|----------------------------------------------------|-------|
| Hydroll R lb./ton                                  | 2.02  |
| Cleaner conc.—per cent $\text{CaF}_2$ assay        | 94.27 |
| Cleaner conc.—per cent $\text{CaCO}_3$ assay       | 5.03  |
| Cleaner conc.—per cent $\text{CaF}_2$ distribution | 68.96 |
| Cleaner tailing—per cent $\text{CaF}_2$ assay      | 63.31 |
| Rougher tailing—per cent $\text{CaF}_2$ assay      | 24.81 |

We claim:

1. A process of beneficiating fluorite-containing ores, which comprises subjecting an aqueous pulp of such ores to froth flotation in the presence of from about 0.2 to 5.0 lbs./ton of ore of a collector comprising a water-soluble product selected from the group consisting of sulfonates of the green acid type obtained in the refining of petroleum lubricating oils and soaps and water-soluble salts of such sulfonates.

2. A process of beneficiating fluorite-containing ores in which a major portion of the gangue is comprised of non-silicious minerals, which comprises subjecting an aqueous pulp of the ore to froth flotation in the presence of an effective amount of a depressant for the non-silicious gangue, about 0.2 to 5.0 lbs./ton of ore of a water-soluble product selected from the group consisting of sulfonates of the green acid type obtained in the refining of petroleum lubricating oils and soaps and water-soluble salts of such sulfonates, and an amount of a compatible oiling agent effective to increase the water-repellant properties of the water-soluble sulfonated product.

3. A process of beneficiating fluorite-containing ores which comprises subjecting an unheated aqueous pulp of such ores to froth flotation in the presence of from about 0.2-5.0 lbs./ton of ore of a collector selected from the group consisting of the water-soluble sulfonates of the green acid type obtained in the refining of petroleum lubricating oils and soaps and water-soluble salts of such sulfonates.

4. A process of beneficiating fluorite-containing ores in which a major portion of the gangue is comprised of non-silicious minerals which comprises subjecting an unheated aqueous pulp of the ore to froth flotation in the presence of an effective amount of a depressant for the non-silicious gangue and about 0.2-5.0 lbs./ton of ore of a collector selected from the group consisting of the water-soluble sulfonates of the green acid type obtained in the refining of petroleum lubricating oils and soaps and water-soluble salts of such sulfonates.

5. A method according to claim 2 in which the oiling-agent is present in amounts of from about 0.2 to 2.5 lbs. per ton of ore.

6. A method according to claim 2 in which the oiling-agent is an unsulfonated petroleum hydrocarbon.

7. A method according to claim 2 in which the oiling-agent comprises an unsulfonated glyceride oil.

8. A method according to claim 2 in which the oiling-agent comprises a fatty-acid.